

April 14, 1931.

E. L. CHAMBERLAIN

1,801,245

PREPARED ROOFING MATERIAL

Filed June 18, 1928



INVENTOR  
Eli L. Chamberlain  
BY *H. L. K. [Signature]*

## UNITED STATES PATENT OFFICE

ELI L. CHAMBERLAIN, OF NORWOOD, MASSACHUSETTS, ASSIGNOR TO BIRD & SON, INC.,  
OF EAST WALPOLE, MASSACHUSETTS, A CORPORATION OF MASSACHUSETTS

## PREPARED ROOFING MATERIAL

Application filed June 18, 1928. Serial No. 286,200.

This invention relates to improvements in what is known as prepared roofing material and has for its object to provide a novel, attractive and more durable material of this character, and may be made either in the form of rolled roofing or as individual or strip shingles.

In the drawings:—

Fig. 1 shows in plan a portion of the roofing material as made in the form of rolled roofing;

Fig. 2 shows a cross-section of the same;

Fig. 3 shows in perspective an individual shingle of a modified type involving additional layers; and

Fig. 4 shows a cross-section of the shingle shown in Fig. 3.

The roofing material and shingle shown in the drawings are of an improved type of composition made up of a wool or rag felt or any other fibrous material saturated in a bituminous compound or any other waterproofing material which penetrates into and through the same so as to render it water resistant.

The base may also be a plastic or metallic in character or a sheet of any suitable material having the desired characteristics. It has long been common to apply to such bases additional asphalt or other coating material and deposit thereon a granular substance such as crushed slate. When, however, the art has attempted to build up the thickness of the shingles or roofing, especially at the butts of shingles, there has been a marked tendency

for the upper portion to slide, and what is called "alligator", when exposed on the roof. The sliding is commonly due to the use of too soft an asphalt coating or too great a thickness of the coating material and when,

in an effort to obviate this, a harder asphalt has been used, it has tended to check, crack or open in fissures, giving the so-called "alligator" appearance. Naturally, a material having the alligator appearance, besides being unsightly, is not as durable, as the sun-light and moisture has a chance to penetrate in the cracks or fissures and the roofing is more readily attacked by the elements.

This invention has particularly to do with the provision of a thick roofing material the

surface of which has no appreciable tendency to slide or alligator, and this result is achieved by introducing into the asphalt coating which receives the granular mineral matter or crushed slate, a suitable quantity of asbestos or other similar fibre, the introduction of which minimizes or prevents sliding and "alligatoring" when used with a suitable bituminous material or other coating.

It was found that when asbestos was mixed with asphalt, the latter became more pliable and more adhesive, especially at low temperatures. For smooth surfaced roll roofings this results in an unusually pliable sheet and for slate surfaced roofings and shingles, it not only adds to the pliability but decreases the tendency to shatter at low temperatures.

Referring to the drawings, and particularly Figs. 1 and 2, 2 indicates a lower or base layer of saturated felt or other fibrous material, and 4 a coating thereon of asphalt-asbestos mixture which in its preferred form consists of from 90 to 95 parts of 18° to 20° penetration, 210° F. to 215° F. melting point asphalt, and 5 to 10 parts by weight of asbestos fibre. The asphaltic material, however, may vary from 75 to 99% with a penetration ranging from 16° to 30° with a melting point variation from 180° F. to 225° F. and the quantity of asbestos may range from 1% to 25%. Upon this layer of asphalt-asbestos compound is placed a surfacing layer of crushed slate or other suitable granular material which is rolled so as to cause the asphalt asbestos compound to well up into the interstices and hold the material firmly. In practice I have found that the asphalt-asbestos compound gives a superior binding to crushed slate as compared with the ordinary bituminous binders heretofore employed.

Referring to Figs. 3 and 4, which show an individual shingle, 2 indicates the saturated felt as before; 5 a surface layer of binder which is preferably asphalt-asbestos compound, but may be of ordinary asphalt; 6 a layer of granular material placed thereon, 7 a layer of asphalt-asbestos compound; and 8 a second layer of crushed slate. It will be noted that the second layer of crushed slate and its binder of asphalt-asbestos compound

has been carried over but a part of the lower or butt end of the original shingle. In this way the shingles are provided with a thickened butt which gives the desired appearance or shadow effect on the roof, and the exposed portions of the shingles are rendered more durable so as to better resist the elements.

Having described my invention, what I wish to claim and secure by Letters Patent is:—

- 10 1. As a new article of manufacture a roofing sheet comprising a base layer having a coating layer thereon consisting of a major portion of bituminous material mixed with a minor portion of inert material and a surface layer of granular mineral matter held to said sheet by said coating.
- 15 2. As a new article of manufacture a roofing material comprising a sheet of suitable material as a base therefor, a bituminous coating thereon including asbestos fiber intermixed with the same, said coating including a major portion of asphaltic material and a minor portion of the asbestos fiber and 25 a surfacing of granular mineral matter partially embedded in said bituminous coating.
- 20 3. As a new article of manufacture, a roofing material comprising a felt base saturated with a bituminous compound, a bituminous coating thereon including asbestos fiber intermixed with the same, said coating including a major portion of asphaltic material and a minor portion of the asbestos fiber and 35 a surface of granular mineral matter partially embedded in said bituminous coating.
- 30 4. As a new article of manufacture a roofing material comprising a sheet of suitable material, as a base therefor, a bituminous coating thereon, a layer of granular material, an additional coating of bituminous compound thereon including asbestos fiber intermixed with the same, said coating including a major portion of asphaltic material and a minor portion of the asbestos fiber and 45 an additional surface coating of granular mineral matter partially embedded in said bituminous coating.
- 40 5. As a new article of manufacture, a roofing material comprising a felt base saturated with a bituminous compound, a bituminous coating thereon, a layer of granular mineral matter, an additional coating of bituminous compound thereon including asbestos fiber intermixed with the same, said coating including a major portion of asphaltic material and a minor portion of the asbestos fiber and 55 an additional surface coating of granular mineral matter partially embedded in said bituminous coating.

60 ELI L. CHAMBERLAIN.